

# UNITED STATES PATENT OFFICE.

JAMES C. DAVIS, OF HINSDALE, ILLINOIS, ASSIGNEE TO AMERICAN STEEL FOUNDRIES,  
OF NEW YORK, N. Y., A CORPORATION OF NEW JERSEY.

## ART OF MOLDING STEEL CASTINGS.

1,165,651.

Specification of Letters Patent. Patented Dec. 23, 1915.

No Drawing.

Application filed March 22, 1915. Serial No. 16,203.

To all whom it may concern:

Be it known that I, JAMES C. DAVIS, a citizen of the United States, and resident of Hinsdale, in the county of DuPage and State of Illinois, have invented certain new and useful Improvements in the Art of Molding Steel Castings, of which the following is a specification.

My invention relates to the art of casting and has particular reference to a novel method of hardening or modifying the face of steel castings.

I am aware that it is a common practice after a mold has been formed to apply a coating or wash to the face thereof, such coating or wash consisting of a carbon-containing mineral, sand and a binder. This practice has been followed in molding steel castings but the resulting product, while having the required hardened exterior, is unsightly and altogether too rough for ordinary use. This condition arose from the combustion of the carbon element thus giving off a gas which in its escape prevented the metal from lying naturally against the face of the mold.

I have conceived of a method of casting whereby I am enabled to secure the desired results as to exterior hardness and at the same time produce a casting which is smooth and sightly. A satisfactory substance is found to be a mixture of a carbonaceous material such as 80% ferro-manganese, silica molding sand and linseed oil, the elements being combined in substantially the following proportions:  $1\frac{1}{2}$  lbs. ferro-manganese,  $\frac{1}{2}$  lb. molding sand,  $\frac{1}{3}$  pint linseed oil. These materials when thoroughly mixed form a plastic substance which I apply to the pattern in the mold; this is covered with the ordinary backing sand and the entire

mold is then rammed with sand in the usual manner after which the pattern is withdrawn and the mold dried as in ordinary dry sand mold practice. After the metal is cast in a mold, such as described, the carbonaceous material is probably ignited as heretofore but the use of the silica molding sand serves to create voids or interstices for the escape of the gases with the result that the face of the casting is smooth.

The exact proportions set forth are not requisite and may be varied to a certain extent in order to carry out the method here disclosed.

It will be understood that the linseed oil acts solely as a binder and that only such quantity need be used as is necessary to bind the particles of sand and carbonaceous material together and retain the imprint of the pattern after the removal thereof from the mold.

I claim:

1. The method of preparing molds which consists in the form of a compound containing carbonaceous material, molding sand and a binder, applying said compound to a pattern, backing the pattern with sand, then ramming the mold, substantially as described.

2. In the art of preparing molds for steel castings, the steps consisting in forming a compound including carbonaceous material, molding sand and a vegetable oil binder, applying the compound to the pattern, backing the compound with sand, then ramming the mold, then stripping the pattern from the mold, substantially as described.

JAMES C. DAVIS.

Witnesses:

A. DUVOR JONES,  
F. J. HEPPelman.

It is hereby certified that in Letters Patent No. 1,165,651, granted December 28, 1915, upon the application of James C. Davis, of Hinsdale, Illinois, for an improvement in "The Art of Molding Steel Castings," an error appears in the printed specification requiring correction as follows: Claim 1, line 2, (line 65 of page,) for the word "form" read *forming*; and that the said Letters Patent should be read with this correction therein that the same may conform to the record of the case in the Patent Office.

Signed and sealed this 18th day of January, A. D., 1916.

[SEAL.]

J. T. NEWTON.

*Acting Commissioner of Patents.*

Cl. 22—190.